

March 23, 1937.

C. S. TREACY

2,074,676

LIGHT SENSITIVE CELL MANUFACTURE

Filed March 6, 1935

FIG. 1



## UNITED STATES PATENT OFFICE

2,074,676

## LIGHT-SENSITIVE CELL MANUFACTURE

Cyril S. Treacy, Scarsdale, N. Y., assignor to  
United Research Corporation, Long Island City,  
N. Y., a corporation of Delaware

Application March 6, 1935, Serial No. 9,584

11 Claims. (Cl. 201—63)

The invention relates to the manufacture of selenium cells of the type shown in the patent to Carpenter, #1,942,958, wherein use is made of a glass support which carries a layer of platinum separated into two electrodes by a sinuous trace. 5 Selenium, or similar light-sensitive material, is sublimed onto and bridges the gap between the adjacent electrode portions.

The present invention relates to an improved process for depositing by sublimation, selenium or similar light-sensitive material on the interdigitated electrodes or grid.

Selenium occurs in several allotrophic forms having different degrees of photo-sensitivity. In subliming selenium, it is desirable to insure, not only that the right kind of crystals are formed on the electrodes, but also that a fine grain deposit of selenium or the like be obtained on the electrodes or grid, as the finer the grain, the more uniformly opaque or dense is the deposit. 15 Also, a finer grain adheres better to the electrodes, which apparently accounts for lower cell noise when using the cell for reproducing sound from sound film.

In my application, Serial No. 9,585, filed March 25, 1935, I have disclosed and claimed certain features disclosed herein for the temperature control of crystal growth to insure that a particular allotrophic form which is photo-sensitive will be crystallized on the electrodes or grid. The present invention relates to a process for insuring that crystals of small size will be obtained.

I have discovered that the grain of the deposit is not as fine when the grid is subjected to selenium vapor for the first time as it is if the initial deposit is removed, for example, by scraping it off the grid with a dull knife, and a second deposit sublimed on the grid. The second deposit also forms more uniformly, and in a shorter time, 35 which is conducive to smaller crystals. The deposition and removal of the crystals are repeated several times, such as six times, with the result that the final coating is deposited uniformly in a short time and with an even layer of crystals so small that the individual crystals are only visible when viewed with a high power objective lens.

Prior to the final deposit, and after the preceding deposit has been scraped away, the metallic electrode surface has been examined, with the result that no visible change in the electrode surface is brought about by the crystallizations and scrapings, the surface appearing smooth even when enlarged four hundred times. In some 50 way which is not understood, the removal of the

crystalline deposit from the grid serves to sensitize the grid surface and facilitate a subsequent deposition of crystals.

For further details of the invention, reference may be made to the drawing, wherein:

Fig. 1 is a side elevation, partly in section, of a furnace which may be employed for subliming selenium or the like onto the electrodes of the cell according to the invention.

Fig. 2 is a perspective view of the furnace of Fig. 1 with the furnace open.

Fig. 3 is a perspective view of a cell element onto which the selenium or the like may be sublimed according to the invention.

A cell element 10, onto which the light-sensitive material is to be sublimed, is shown in Fig. 3, wherein the glass support 1, has the interdigitated electrodes or grid 2, 3. This grid 2, 3 may be made as follows, or otherwise:

Preferably, the glass support 1 for the grid 2, 3 is soft glass. The glass support 1 is coated with a metallic solution, such as a colloidal mixture of two parts of platinum chloride and one part of gold chloride, and fired in a muffle furnace not shown. In some cases, the surface of the fused metallic layer on the glass may be uneven or warped, due to raising the soft glass to a temperature high enough to fuse the metal to it. In other cases, the grid blank is not warped. Preferably, the metal layer is pre-fired to a temperature below the fusion point. After cooling, the hard coating on the metal is dissolved in water, the sinuous trace 4, which may be 1 or 2 mils wide, is then cut, and thereafter the grid 2, 3 is fired to a temperature to fuse the metallic grid 2, 3 to the glass 1, as described and claimed in my co-pending application, Serial No. 9,583, filed March 6, 1935.

The element 10 is now ready to have selenium or the like sublimed on it according to the present invention, and for this purpose, use may be made of a furnace such as shown in Figs. 1 and 3. This furnace comprises a hot plate 5, which supports the cell elements 10, and a second hot plate 6, which carries a molten pasty layer 7 of the selenium or other light-sensitive material to be sublimed onto the elements 10. The plates 5 and 6 are hinged at 8 whereby the upper plate 6 overlies the bottom plate 5 when the oven is closed, as in Fig. 1, these plates being held apart by a distance of the order of  $\frac{1}{16}$  inch to  $\frac{1}{4}$  inch, this distance of course being determined by the height of the insulating spacer 9. The plate 5 is provided with a thermometer 11, an electric heater 12 and a thermostat generally indicated at 13. The 55

upper plate 6 is similarly provided with a thermometer 14, an electric heater 15, and a thermostat control indicated at 16.

When the furnace in Fig. 3 is fully opened, the 5 subliming surface 6 is horizontal, and in this position, it is sprinkled, while hot, with a thin coating of the subliming mixture which may, for example, comprise 19 parts of pure powdered selenium intimately ground with one part of powdered tellurium. The subliming surface 6 at this time should have a temperature of about 245° C. or higher, preferably 295° C., whereby the subliming mixture melts to form a pastry coating on surface 6 as indicated at 7. The furnace is now closed as 10 shown in Fig. 1, the lower plate 5 being maintained by thermostat 13 at a temperature such that the elements 10 are kept below the melting point of the subliming mixture 7, while the temperature of the upper plate or subliming surface 6 is regulated by thermostat 14 to a temperature such that 15 a heavy concentration of vapor from mixture 7 is provided for coating the elements 10.

The lower plate 5 is provided with a series of apertures 17 at opposite sides thereof. These 20 apertures 17 in effect provide vanes to cool the lower plate 5 and prevent its temperature from rising above the desired value due to its proximity to the upper plate 6.

For the initial sublimed coating, the subliming 25 surface 6 is regulated at a temperature of 245° C. or higher, preferably 295° C., depending on the desired rate of evolution of vapor, and the lower plate 5 is regulated to a temperature of 140 to 145° C., whereby the elements 10 receive the vapor 30 at the correct temperature for the growth of the particular allotropic form which is photo-sensitive. The feature of temperature control to control crystal growth is disclosed and claimed in my copending application, Serial No. 9,585, filed 35 March 6, 1935. The sublimation proceeds for about one to one and one-half hours and results in a soft sublimed coating which is easily scraped off the elements 10. When the elements 10 are fairly well coated, as they will be under the conditions 40 above mentioned, they are removed from the furnace and scraped with a dull knife to thoroughly remove the sublimed coating on the electrodes 2, 3. If the elements 10 are flat, a flat scraper may be used; if they are warped as shown 45 in Fig. 2, a curved scraper is used. The scraped elements 10 are replaced in the furnace and again the mixture 7 is sublimed on them, whereupon the sublimed coating is again scraped off. The steps of coating and scraping are repeated five 50 or six times, the time of coating being successively reduced as the formation of a subsequent layer is hastened by the former crystallization of sublimations. After the selenium has been deposited and scraped away about six times, the grid surface is 55 thoroughly cleaned with a jeweler's brass bristle brush, or the like, to remove all visible portions of the sublimed material, and the final coating of the selenium mixture is sublimed on the grid element 10.

The final coating is always done with a fresh 60 charge of subliming mix 7 on the upper subliming surface, the previous mixture 7 having been removed from surface 6, as it has been found that the use of old mix gives cells with a lower output. This is undoubtedly due to the formation of oxides in the mix. The top stove 6 is kept at 325° C., 65 which is higher than used in the pre-coatings, while the bottom stove 5, on which the grids 10 rest is kept at 140°. A 4½ minute period is gen-

erally sufficient to deposit a non-transparent closely adherent and fine grained deposit.

After removing the grids 10 from the furnace, the deposit of sublimed material on the surface of the electrodes 2, 3, outside of the grid 4, is scraped away and two drops of a dilute solution of iodine in carbon disulphide is used to wet the deposit. The iodine possibly reacts with traces of oxide, present to reduce it to selenium and tellurium. Excess iodine forms selenium and tellurium iodide 10 which tends to decompose, and also to sublime away, and care must therefore be taken not to use too much. This treatment apparently produces cells with better signal to noise ratio.

Subsequent annealing of the coated grids is 15 not necessary, as the desired photo-sensitive form of the light-sensitive material is originally formed on the grids, due to maintaining the lower plate 5 at the temperature necessary for the desired 20 crystal growth.

A protective glass cap is cemented over the trace 4, the excess selenium around the cap is removed, and the element mounted, for example, as shown and claimed in the application to Carpenter et al., Serial No. 747,610, filed October 9, 1934, for 25 "Light-sensitive cell", or as in the patent to Lyon, #1,948,766.

I claim:

1. The method of obtaining a fine grain opaque 30 coating of selenium on separated electrodes which comprises maintaining said electrodes at an elevated temperature favorable for the formation of photo-sensitive crystals while directing vapor of selenium thereon for a certain time, removing the material thus deposited on said electrodes, and thereafter maintaining said electrodes at said elevated temperature, while directing vapor of selenium thereon for a shorter time.

2. The method according to claim 1, wherein 40 said first-mentioned directing of vapor continues for a period of the order of an hour, and said last-mentioned directing of vapor continues for a period of the order of a few minutes.

3. The method of obtaining a fine grain opaque 45 coating of selenium on separated electrodes which comprises maintaining said electrodes at a temperature of about 140 to 145° C., while directing selenium vapor thereon at a certain rate for a certain time, removing the selenium thus deposited thereafter maintaining said electrodes at said 50 temperature while directing selenium vapor thereon for a shorter time.

4. The method of sensitizing a metallic surface 55 to deposition of selenium thereon by sublimation which comprises subliming selenium on said surface and removing the selenium thus sublimed.

5. The method according to claim 4 which comprises effecting said removing by scraping.

6. The method of coating selenium on separated electrodes which comprises sensitizing said 60 electrodes by maintaining said electrodes at an elevated temperature favorable for the formation of photo-sensitive crystals while directing vapor of selenium thereon for a certain time and removing the selenium thus deposited; and thereafter directing vapor of selenium on said electrodes.

7. The method according to claim 6 wherein 65 said last mentioned directing of selenium vapor is effected while maintaining said electrodes substantially at said elevated temperature.

8. The method according to claim 6 which comprises repeating said sensitizing prior to said last step of directing selenium vapor on said electrodes.

9. The method according to claim 6 which comprises effecting said removing by scraping.

10. The method of coating selenium on separated electrodes which comprises sensitizing said electrodes by maintaining said electrodes at an elevated temperature favorable for the formation of photo-sensitive crystals while directing vapor of selenium thereon for a certain time and scraping the selenium thus deposited; repeating said sensitizing, and thereafter directing vapor of fresh selenium on said electrodes while maintaining said electrodes substantially at said elevated temperature.

11. The method of coating selenium on a sur-

face which comprises sensitizing said surface by maintaining said surface at an elevated temperature favorable for the formation of photo-sensitive crystals while directing vapor of selenium thereon for a certain time, said deposited selenium having a certain grain size, removing the selenium thus deposited, again directing vapor of selenium on said surface, said second deposit of selenium having a finer grain size than said first deposit, and repeating the foregoing steps until the selenium has the fineness of grain desired.

5

10

CYRIL S. TREACY.

CERTIFICATE OF CORRECTION.

Patent No. 2,074,676.

March 23, 1937.

CYRIL S. TREACY.

It is hereby certified that error appears in the printed specification of the above numbered patent requiring correction as follows: Page 2, first column, line 13, for "pastry" read pasty; and second column, line 75, claim 1, for "material" read selenium; and that the said Letters Patent should be read with these corrections therein that the same may conform to the record of the case in the Patent Office.

Signed and sealed this 25th day of May, A. D. 1937.

(Seal)

Henry Van Arsdale  
Acting Commissioner of Patents.

9. The method according to claim 6 which comprises effecting said removing by scraping.

10. The method of coating selenium on separated electrodes which comprises sensitizing said electrodes by maintaining said electrodes at an elevated temperature favorable for the formation of photo-sensitive crystals while directing vapor of selenium thereon for a certain time and scraping the selenium thus deposited; repeating said sensitizing, and thereafter directing vapor of fresh selenium on said electrodes while maintaining said electrodes substantially at said elevated temperature.

11. The method of coating selenium on a sur-

face which comprises sensitizing said surface by maintaining said surface at an elevated temperature favorable for the formation of photo-sensitive crystals while directing vapor of selenium thereon for a certain time, said deposited selenium having a certain grain size, removing the selenium thus deposited, again directing vapor of selenium on said surface, said second deposit of selenium having a finer grain size than said first deposit, and repeating the foregoing steps until the selenium has the fineness of grain desired.

5

10

CYRIL S. TREACY.

CERTIFICATE OF CORRECTION.

Patent No. 2,074,676.

March 23, 1937.

CYRIL S. TREACY.

It is hereby certified that error appears in the printed specification of the above numbered patent requiring correction as follows: Page 2, first column, line 13, for "pastry" read pasty; and second column, line 75, claim 1, for "material" read selenium; and that the said Letters Patent should be read with these corrections therein that the same may conform to the record of the case in the Patent Office.

Signed and sealed this 25th day of May, A. D. 1937.

(Seal)

Henry Van Arsdale  
Acting Commissioner of Patents.

CERTIFICATE OF CORRECTION.

Patent No. 2,074,676.

March 23, 1937.

CYRIL S. TREACY.

It is hereby certified that error appears in the printed specification of the above numbered patent requiring correction as follows: Page 2, first column, line 13, for "pastry" read pastry; and second column, line 75 claim 1, for "material" read selenium; and that the said Letters Patent should be read with these corrections therein that the same may conform to the record of the case in the Patent Office.

Signed and sealed this 25th day of May, A. D. 1937.

(Seal)

Henry Van Arsdale  
Acting Commissioner of Patents.